

## UNITED STATES PATENT OFFICE

JOHN R. CAIN, OF WASHINGTON, DISTRICT OF COLUMBIA, AND SAMPSON W. YATES, OF CINCINNATI, OHIO, ASSIGNEES TO THE RICHARDSON COMPANY, OF LOCKLAND, OHIO, A CORPORATION OF OHIO

## IRON SULPHIDE MATERIAL AND PROCESS OF MAKING THE SAME

No Drawing.

Application filed April 16, 1928. Serial No. 270,571.

Our invention relates to the production of castings containing iron sulphide which can be used with advantage in a soluble anode process of forming electrolytic iron with progressive maintenance of a condition of negligible hydrogen ion concentration in the electrolyte.

It is the object of our invention to provide an anode for the purpose named from readily obtainable ores, with the minimum of expense, and using as little heat as possible.

Specifically it is our object to form anodes as bodies cast from material formed by heating together iron oxide (hematite ore) and iron di-sulphide (pyrite), both of which are plentiful minerals.

The equipment used by us may be a cupola or shaft furnace which is economical to build and operate, lined preferably with refractories which will not be corroded by ferrous sulphide at the melting zone, magnesia, or a neutral lining such as carborundum, giving good results.

In describing our process we will give the best procedure as now followed by us, it being understood that this is merely indicative of one mode of shop practice which is available. By using a coke similar to blast furnace coke we obtain furnace flue gases which are valuable for combustion and generation of heat for annealing and other furnaces. By close regulation of air supply using cupola foundry coke we may also obtain a combustible flue gas.

A special fuel is not required in our process, and it should be noted that a considerable proportion of the iron bearing constituents of the charge do not require reduction to iron. Also, the reaction which is induced where one atom of Fe, obtained from reduction of the hematite ore, combines with one of the atoms of sulphur in the pyrite ( $FeS_2$ ) giving two molecules of  $FeS$ , produces a definite amount of exothermic heat, which assists in making the melt and maintaining the temperature of the reaction products above the melting point. The resulting molten iron sulphide can be tapped either into molds or into a ladle from which the molds are filled.

The air supply to our furnace may be pre-heated with any waste energy such as is obtained from the stack gases, but that is non-essential and we obtain ferrous sulphide material using a cold air blast, at a temperature sufficiently above the melting point for proper pouring and casting.

We prepare the ores of hematite and pyrite in finely divided form, and mix them with reaction coke using a binder which will permit of briquetting. This helps to avoid loss of sulphur through the stack.

In starting a run we charge the cupola with coke, which is ignited. When the shaft is hot, the coke layer is covered with briquets, then with a further layer of coke, then layers of briquets and coke alternately.

We get best results by using in the briquets enough of the iron pyrite to result in a slight excess of sulphur over what would be required to give the exact combining weights.

We find that we get good results by using some surplus reaction coke over the proper combining weight.

We find it preferable to control the air blast, and to measure both the rate of flow and the pressure thereof. The blast will vary, of course, with the furnace and the fuel, and the operator will find it advisable not to drive the furnace to the point of producing in it a strongly oxidizing atmosphere, as this promotes loss of sulphur, as  $SO_2$  in the flue gases. We have been able to control loss of sulphur through control of the blast.

The expenditure of heat to make a given charge of iron as iron-sulphide is theoretically about fifty per cent of what would be required to produce an equivalent weight of molten pig iron, because only about 50% of the total iron in the furnace requires reduction.

The furnace may have a floor of, for instance, molding sand, upon which will collect a thin iron-silicate-sulphide skin. Above this skin the molten  $FeS$  will collect.

Further, we may secure molten material which is essentially a solid solution of iron oxides and iron sulphides, and this mate-

rial gives good results as anodes. Methods of producing these and other anode materials form the subject of other patent applications.

5. The iron sulphide material will solidify in the molds into solid anodes; these can be cast with terminal rods of iron in them, if desired.

By crushing the ores and coke to 20 mesh size, we obtain a good yield. With a furnace lining of magnesia refractory we have but little cutting of the furnace walls, and the slag is easily handled.

As a flux we may use fluor-spar by itself or together with fluxing materials of low cost. Using fluor-spar by itself, the sulphur in the slag is below one per cent, while with ordinary calcium carbonate limestone by itself the slag contains large proportions of sulphur.

The slag floats upon the molten ferrous sulphide in the well of the furnace and is tapped off.

The product of our invention so far as its physical properties are concerned is improved considerably as a cast body by a suitable heat treatment and Sampson W. Yates, one of the co-inventors herein is making application for patent of even date herewith for heat control and treatment of our product, and the resultant improved product thereby obtained by him.

When used as anode material, in a ferrous chloride electrolyte, the cast products of our process inhibit the formation of ferric salts by electrolytic action, and thus avoid the formation of acids and the development of harmful hydrogen ion concentration. They further tend directly to neutralize any acid present. The anodes hold their shape as they are dissolved and require very little cleaning.

Having thus described our process and product, what we claim as new and desire to secure by Letters Patent, is:—

1. That process of producing iron sulphide material, which consists in heating iron ore and pyrite together with a separate reducing agent for iron ore in the presence of burning fuel, with the result of the iron in said ore taking on an atom of sulphur, thus converting the mass mainly into iron sulphide, the temperature of the heating being sufficient to fuse the iron sulphide and any slag formed and then tapping off the molten material.

2. That process of producing iron sulphide material, which consists in forming briquets of finely divided iron ore, pyrite and carbon, heating said briquets in a shaft furnace, in the presence of burning fuel and tapping off the resultant material which is mainly iron sulphide the temperature of the heating being sufficient to fuse the iron sulphide material.

3. That process of producing iron sulphide material, which consists in forming briquets of finely divided iron ore, pyrite and carbon, heating said briquets in a shaft furnace, the temperature of the heating being sufficient to fuse ferrous sulphide; and tapping off the resulting material which is mainly iron sulphide, and using a flux in the process of a type which will not take up sulphur or iron.

4. A process for producing ferrous sulphide material, which consists in placing iron ore, pyrite and carbon, together with fuel and flux in a shaft furnace, heating the products using a blast regulated to oxidize a minimum of sulphur, with the result of the formation of molten ferrous-sulphide material the temperature of the heating being sufficient to fuse the ferrous sulphide material; and flowing the molten material into molds.

5. A process for producing ferrous sulphide material which consists in causing oxide iron ore, pyrites and carbon to react together in the presence of burning fuel to produce molten ferrous sulphide material and a slag.

6. A process for producing ferrous sulphide material which comprises comminuting and mixing a material containing ferric sulphide, a material containing a reducible compound of iron and a carbonaceous reducing agent, and heating the mixed materials in the presence of burning solid carbonaceous fuel to a temperature sufficient to melt the reaction products and in the presence of a flux, whereby the molten material containing ferrous sulphide and a molten slag is produced, and tapping off the ferrous sulphide material.

7. A process for producing molten ferrous sulphide material which comprises mixing a material containing ferric sulphide, a material containing a reducible compound of iron, and a carbonaceous material, and charging said material with flux comprising fluorspar into a furnace, and heating said substances in the presence of burning fuel to a temperature sufficient to fuse the products of reaction, and separating the resulting fused ferrous sulphide material from the fused slag.

JOHN R. CAIN.  
SAMPSON W. YATES.

120

125

130